

1

3,394,984

IODINATION OR HYDROIODINATION OF ALKYLENE BISAMIDE-CONTAINING POLYPROPYLENE FIBERS DYED WITH BASIC DYES  
Akio Koshino and Hirohisa Nara, Uji-shi, Kyoto-fu, Japan, assignors to Nippon Rayon Co., Ltd., Kyoto-fu, Japan  
No Drawing. Continuation of application Ser. No. 251,487, Jan. 15, 1963. This application Feb. 7, 1967, Ser. No. 614,518  
6 Claims. (Cl. 8—31)

The present application is a continuation of S.N. 251,487, filed Jan. 15, 1963, now abandoned.

The present invention relates to a process for improving the light fastness of dyed polymeric olefines.

In general, brilliant shades are obtained by basic and cation dyestuffs, but the light fastness of the dyed products is not satisfactory. Accordingly, when above dyestuffs are used, dyed synthetic fibres and other articles formed of polymeric olefines possess extremely low light fastness, so that these dyestuffs cannot be used in practice.

As the result of extensive investigations to improve the light fastness of polymeric olefines which are dyed with basic and cation dyestuffs and to bring these dyed polymeric olefines into practical use, it has now been found that the addition of iodine into a dyebath or the after-treatment of dyed polymeric olefines with iodine or with hydrogen iodide provides a marked improvement in the light fastness of polymeric olefines which are dyed with above dyestuffs and also acid dyestuffs.

According to the feature of the present invention, a process for improving the light fastness of dyed polymeric olefines comprises dyeing the polymeric olefines in a dye bath containing iodine or hydrogen iodide as an auxiliary agent.

According to the another feature of the present invention, therefore, a process for improving the light fastness of dyed polymeric olefines comprises after-treating the dyed polymeric olefines with iodine or hydrogen iodide.

The method for improving the dyeing properties of polyolefine fibres by treating them with iodine is known, but in the present invention iodine is used for improving the light fastness of dyed polymeric olefines which are dyed with basic, cation or acid dyestuffs.

Consequently, the present invention is different from the prior method for the pre-treatment of polymeric olefines with iodine in that the object of the present invention is to improve the light fastness of the dyed product and the object of the prior method is to improve dyeability.

The synthetic fibres and other articles herein referred to as being formed of polymeric olefines included those produced of polyolefines alone, mixtures of polyolefines and other polymers, mixtures of polyolefines and organic compounds having lower molecular weight, graft polymers based on polyolefines, and copolymers of polyolefines with other compounds.

Treatments with other halogens and halogenides except iodine and hydrogen iodide give little effect to improve the light fastness of polymeric olefines dyed with basic and cation dyestuffs. Further, treatments with other compounds which are known as lightproof agents such as benzophenone, benztriazol and their derivatives give also no effect to improve the light fastness of polymeric olefines dyed with basic, cation or acid dyestuffs.

Although the mechanism how the light fastness of dyed polymeric olefines treated with iodine or hydrogen iodide is improved is not clear, it may be considered that iodine or hydrogen iodide in said fibres or other articles absorbs energy of sunlight and prevent the decomposition of basic, cation dyestuffs, etc.

2

In case iodine or hydrogen iodide is used as an auxiliary agent during dyeing process in the present invention, for example, synthetic fibres or other articles based on polymeric olefines are dyed in a bath containing requisite amounts of basic dyestuff and 0.5—15% of iodine based on the weight of fibres. In this case, iodine is previously dissolved with a suitable solvent, and then added to the dye bath. Dyeing is carried out at a given pH and 100° C. for 0.5—2 hours, and the dyed polymeric olefines obtained have very excellent light fastness.

In case dyed polymeric olefines are subjected to the after-treatment with iodine or hydrogen iodide in the present invention, for example, synthetic fibres or other articles formed of polymeric olefines dyed with basic or cation dyestuffs are treated in the bath, in which iodine or hydrogen iodide is dissolved in water, alcohol, chloroform or an aqueous solution of potassium iodide, at a temperature higher than room temperature for from several minutes to 2 hours and then rinsed sufficiently. Further, this treatment can be carried out in iodine or hydrogen iodide vapour.

The present invention can be applied in case the polymeric olefines are dyed with basic, cation or acid dyestuffs after chemical treatment, such as chlorination, sulfonation and acid and amine treatments.

The light fastness of dyed polymeric olefines subjected to the after-treatment is outstandingly superior into that of the untreated products. For example, if the light fastness of polymeric olefines dyed with basic dyestuffs is only grade 1 according to AATCC test when untreated, it becomes grade 4, 5, 6 or higher after being treated in accordance with one of the processes described above.

The following examples serve to illustrate the present invention, but they are not intended to limit it thereto.

#### EXAMPLE 1

Crystalline polypropylene material having an average molecular weight of 77,000 was blended with 3% by weight of octadecylamine and methylene bis-stearamide respectively and subsequently drawn at a draw ratio of 5 after being melt-spun at 240° C. The resulting fibre was treated with a bath of 20% hydrochloric acid solution at 100° C. for 30 min., neutralized with sodium carbonate solution and then rinsed with cold water sufficiently. The fibre, thus treated, was dyed in a weak alkaline bath containing the basic or cation dyestuffs described in Table I at 100° C. for 60 min. After being treated in a bath containing 5% (based on the weight of fibres) of iodine dissolved in 10 g./l. aqueous potassium iodide solution at 90° C. for 30 min., the dyed materials were rinsed sufficiently and then soaped.

The light fastness of the dyed materials after the above treatment with iodine was greatly improved in comparison with untreated materials as shown in Table I. The light fastness values in Table I are estimated by AATCC test using a Fade-Ometer.

TABLE I

|    | Dyestuff                                                | Light fastness of dyed materials treated with iodine (class) | Light fastness of dyed materials untreated (class) |
|----|---------------------------------------------------------|--------------------------------------------------------------|----------------------------------------------------|
| 60 | Auromine (C.I. Basic Yellow 2) C.I. 41,000              | 4                                                            | 1                                                  |
| 65 | Astra Phloxine FF conc. (C.I. Basic Red 12) C.I. 48,070 | 5                                                            | 1                                                  |
|    | Malachite Green (C.I. Basic Green 4) C.I. 4,200         | 4                                                            | 1                                                  |
|    | Victoria Pure Blue BOH (C.I. Basic Blue 7) C.I. 42,595  | 4                                                            | 1                                                  |
|    | Crystal Violet (C.I. Basic Violet 3) C.I. 42,555        | 5                                                            | 2                                                  |
| 70 | Astrazon Yellow GRL                                     | 5                                                            | 2                                                  |
|    | Astrazon Orange R (C.I. Basic Orange 22) C.I. 43,040    | 4                                                            | 1                                                  |
|    | Astrazon Black M                                        | 5                                                            | 1                                                  |

Crystalline polypropylene material having an average molecular weight of 77,000 was blended with 5% by weight of polyetherester resin prepared from mixture of hydroxy benzoic acid, dimethyl terephthalate and ethylene glycol, and subsequently drawn at a draw ratio of 5, after being melt spun at 270° C.

The fibre thus obtained was dyed in a weak alkaline bath containing 5% (based on the weight of fibre) of iodine dissolved in 10 g./l. of potassium iodide solution and basic and cation dyestuffs described in Table II at 100° C. for 60 min.

The light fastness of the materials thus dyed was greatly improved in comparison with materials dyed without the addition of iodine to the dye bath as shown in Table II. The light fastness values in Table II are estimated by AATCC test using a Fade-Ometer.

TABLE II

| Dyestuffs                                    | Light fastness of materials dyed with the addition of iodine (class) | Light fastness of materials dyed without the addition of iodine (class) |
|----------------------------------------------|----------------------------------------------------------------------|-------------------------------------------------------------------------|
| Auramine OH (C.I. Basic Yellow 2)            | 4                                                                    | 1                                                                       |
| Astra Philoxine FF conc. (C.I. Basic Red 12) | 5                                                                    | 1                                                                       |
| Malachite Green (C.I. Basic Green 4)         | 4                                                                    | 1                                                                       |
| Crystal Violet (C.I. Basic Violet 3)         | 5                                                                    | 2                                                                       |
| Astrazon Orange R (C.I. Basic Orange 22)     | 4                                                                    | 1                                                                       |
| Astrazon Red 6B                              | 4                                                                    | 1                                                                       |

## EXAMPLE 3

After being treated with solution containing calcium hypochlorite and hydrochloric acid, polypropylene fibre was dyed in a weak alkaline bath containing basic or cation dyestuffs, as shown in Table III. The dyed material was subsequently treated in an aqueous solution of 5% of iodine (based on the weight of the fibres) and 25% of potassium iodide (based on the weight of the fibres) at 90° C. for 30 min., rinsed sufficiently and soaped.

The light fastness of the dyed materials, after being treated as described above, was greatly improved in comparison with untreated dyed materials as shown in Table III. The light fastness values in Table III are estimated by AATCC test using a Fade-Ometer.

TABLE III

| Dyestuffs                                  | Light fastness of dyed materials treated with iodine (class) | Light fastness of dyed materials untreated (class) |
|--------------------------------------------|--------------------------------------------------------------|----------------------------------------------------|
| Malachite Green (C.I. Basic Green 4)       | 4                                                            | 1                                                  |
| Victoria Pure Blue BOH (C.I. Basic Blue 7) | 4                                                            | 1                                                  |
| Astrazon Yellow GRL                        | 5                                                            | 2                                                  |
| Astrazon Orange R (C.I. Basic Orange 22)   | 4                                                            | 1                                                  |

## What is claimed is:

1. A process for improving the light fastness of polypropylene fibers blended with an alkylene bis-fatty acid amide dyed with a basic dyestuff which comprises treating said fibers with an aqueous solution containing 0.5-15% of iodine or hydrogen iodide.
2. A process according to claim 1, in which said polypropylene fibers are treated with said solution during dyeing with the basic dyestuff.
3. A process according to claim 1, in which said polypropylene fibers are treated with said solution after dyeing with the basic dyestuff.
4. A process according to claim 1, further comprising treating said polypropylene fibers with an aqueous solution of potassium iodide during application of said iodine or hydrogen iodide solution.
5. A process according to claim 4, in which the concentration of potassium iodide in said aqueous solution is 10 grams per liter.
6. A process according to claim 1, in which, when said member of said group is iodine, the concentration thereof in said solution is from 0.5-15% based on weight of polypropylene fibers.

## References Cited

## UNITED STATES PATENTS

- |           |        |                 |          |
|-----------|--------|-----------------|----------|
| 2,276,951 | 5/1942 | Fisher          | 205-163  |
| 2,537,627 | 1/1951 | Weissart et al. | 260-45.7 |
| 2,805,960 | 9/1957 | Wolinski        | 117-38   |
| 2,931,296 | 4/1960 | Ryan et al.     | 8-100    |

## FOREIGN PATENTS

- |           |        |          |
|-----------|--------|----------|
| 1,083,651 | 6/1960 | Germany. |
|-----------|--------|----------|

## OTHER REFERENCES

Meili: American Dyestuff Reporter, May 1948, pages 81-83, TP890 512.

Diserens: Chemical Technology of Dyeing and Printing, vol. 2, page 84, pub. 1951 by Reinhold Pub. Corp., N.Y.C. TP893D49.

Venkataraman: The Chemistry of Synthetic Dyes, vol. I, page 69, pub. 1952 by Academic Press Inc., N.Y.C. TP913V4C2.

Finch: Fibers and Plastics, January 1960, pages 14-16.

Musgrave: Fibers and Plastics, August 1960, pages 241-244.

Strobel et al.: American Dyestuff Reporter, Aug. 7, 1961, pages 583-585.

NORMAN G. TORCHIN, Primary Examiner.

DONALD LEVY, Assistant Examiner.